

## UNITED STATES PATENT OFFICE

2,518,438

## PROTECTIVE COATINGS

Helen Sellei Beretvás, Chicago, Ill., assignor to  
Nox-Rust Corporation, a corporation of Illinois

No Drawing. Application November 5, 1945,  
Serial No. 626,916

11 Claims. (Cl. 106—267)

## 1

This invention relates to protective coatings for surfaces and more particularly to protective coatings for metallic surfaces to reduce oxidation or corrosion thereof.

The principal object of this invention is to provide an improved protective coating for surfaces which may be readily applied as by spraying, dipping or brushing, which readily and closely adheres to the surfaces for giving maximum protection, which readily dries and does not remain tacky, which does not chip or chalk or peel off after being applied, which is transparent and substantially colorless so that the nature of the coated surfaces may be observed, which does not require removal before the surfaces are subsequently painted or lacquered, and which reacts with the subsequently applied paint or lacquer to form a close bond between the paint or lacquer and the surfaces.

More specifically an object of this invention is to provide an improved protective coating for surfaces comprising soaps formed from metals and two types of organic acids, carried by a suitable carrying vehicle for application to the surfaces to be coated and protected.

A further object of this invention is to provide an improved protective coating for surfaces, comprising soaps, formed from at least two types of metals and two types of organic acids, carried by a suitable carrying vehicle for application to the surfaces to be coated and protected.

Another object of this invention is to include in such protective coatings an inhibitor compound for further deterring the oxidation or corrosion of the coated surfaces.

This invention utilizes metal soaps formed from metals and two different organic acids.

One of the organic acids is a non-drying acid, and naphthenic acid has been successfully utilized. A metal soap is formed by combining metals with this non-drying type organic acid and copper, magnesium, calcium, zinc, strontium, barium, tin, lead, chromium, manganese, iron, cobalt or nickel have been successfully combined with naphthenic acid to form those metal naphthenate soaps.

The other organic acid is an acid, having a relatively high iodine value, such as tall oil acid, rosin acids and tun oil acid. A metal soap is formed by combining metals with these type organic acids and copper, magnesium, calcium, zinc, strontium, barium, tin, lead, chromium, manganese, iron, cobalt and nickel have been successfully combined with tall oil acid to form those metal tall oil soaps.

## 2

One or more metal soaps from each of these groups are mixed together in a suitable carrying vehicle which acts as a solvent for the soaps. A suitable carrying vehicle which has been successfully utilized for the different soaps comprises neutral spirits alone or neutral spirits in combination with a mineral oil.

In mixing the different soaps in the carrying vehicle the different soaps may have the same 10 metals or different metals. For example, lead tall oil soap may be mixed with lead naphthenate soap, or lead tall oil soap may be mixed with zinc naphthenate soap and calcium naphthenate soap.

These mixtures of soaps in the carrying vehicle 15 are liquid in form and may be readily applied to surfaces to be protected, as by spraying, dipping or brushing. After the liquid has been applied to the surfaces, it dries quite rapidly into a tough resin-like protective coating which does not chip or chalk or peel off the surfaces. It is believed 20 that during the drying process a polymerization occurs producing polymers which produce the tough resin-like protective coating. It is found that the dried coating is very difficult to remove by conventional cleaning procedures.

The protective coating is transparent and substantially colorless, although slight coloring may be present depending upon the metals utilized. For example, cobalt in the soaps produces a slight 30 greenish or bluish tint to the coating. If desired, the transparent coatings may be tinted or dyed to provide a coating of pleasing color. The transparent coating enables one to observe the nature or character of the surfaces below the 35 coating.

The soaps being formed of organic acids including naphthenic acid (a petroleum product) causes the protective coating to adhere tenaciously to the coated surfaces thereby providing maximum protection for the coated surfaces. In some 40 instances, the addition of mineral oil in the carrying vehicle also assists in the adhering qualities of the protective coating.

Since the protective coating has drying characteristics and includes metals, it bonds readily 45 with paints or lacquers subsequently applied and therefore forms a good base for the paints and lacquers.

The character of the protective coating, such as toughness, adhesion, thickness, speed of drying, and resistance to heat, humidity, salt spray and salt water immersion, may be controlled by the proper selection of soaps and relative proportions of the ingredients utilized.

In order to further deter the oxidation or corrosion of the coated surfaces an inhibitor of barium base oil, which is a mixture of mineral oil and barium soap utilizing oxidized petroleum for the fatty acid, has been successfully used in this combination. A further inhibitor known commercially as "Lubrizol 738" has been successfully utilized in combination with the barium base oil to assist the inhibiting characteristics of the latter. These inhibitors when combined with the other ingredients of the protective coatings do not alter the above mentioned characteristics thereof but enhance them by further deterring oxidation or corrosion of the coated surfaces. Here then, for the first time there is provided a protective coating of this character having an oxidation or corrosion inhibitor which is transparent and substantially colorless.

While the applied protective coating dries quite rapidly, it may be subjected to heat, infrared rays or ultraviolet rays for accelerating the drying action without impairing the protective coating.

In order to further disclose this invention the compositions of several very successful protective coatings are, by way of example, set forth in detail below and the various protective coatings are designated by the letters A to F, respectively.

|                                               | A        | B        | C        | D        | E        | F        |
|-----------------------------------------------|----------|----------|----------|----------|----------|----------|
| Soaps                                         | Per cent | Per cent | Per cent | Per cent | Per cent | Per cent |
| Zinc naphthenate-8% zinc                      | 5        |          |          |          |          | 10       |
| Calcium naphthenate-5% calcium                | 10       |          | 20       |          |          |          |
| Cobalt naphthenate-6% cobalt                  |          | 10       |          | 20       | 10       |          |
| Lead-Tall Oil-30% lead                        | 10       | 15       | 20       | 30       | 30       | 30       |
| Vehicle                                       |          |          |          |          |          |          |
| Mineral oil—1200 S. U. S. @ 100° F. viscosity | 5        | 5        | 10       | 10       | 10       |          |
| Spirits                                       | 70       | 70       | 40       | 40       | 42       | 50       |
| Inhibitor                                     |          |          |          |          |          |          |
| Barium oil base                               |          |          |          |          | 5        | 10       |
| Lubrizol 738                                  |          |          |          |          | 3        |          |

The protective coatings of A and B are of medium thickness and are thinner than the heavy protective coatings of C through F. This is due to the fact that the relative percentages of soaps and carrying vehicles in the liquid mixture differ. The solid contents of A and B are less than the solid contents of C through F thereby providing thinner protective coatings.

Protective coatings of light thickness may be produced by adding spirits to the above liquids to obtain thinner liquids. For example, the thinner liquids for producing light protective coatings have been successfully obtained by mixing the liquids of A or B with spirits, in the proportions of 20% liquids of A or B and 80% spirits.

Each of the protective coatings, whether light, medium or heavy, give adequate surface protection for their intended purposes and generally speaking the thicker or heavier the protective coating the longer it remains effective. The various protective coatings have successfully protected surfaces from corrosion when subjected to high relative humidities, salt sprays, salt water immersions and tap water immersions for a number of days, and it is found, generally, that the heavier the protective coating the greater the number of days that protection is afforded.

While separate metal soaps have been described as being mixed in the carrying vehicle,

the soaps may be simultaneously formed as by simultaneously reacting one or more metals having basic oxides with the two different acids.

Although the invention has been described with certain illustrated formulas, it will be apparent that changes and modifications may be readily made without departing from the spirit and scope of the invention.

I claim as my invention:

1. A liquid mixture for producing a resin like protective coating for surfaces consisting essentially of at least 2 percent of a metal naphthenate soap formed from naphthenic acid and a metal of the group of copper, magnesium, calcium, zinc, strontium, barium, tin, lead, chromium, manganese, iron, cobalt and nickel, a metal tall oil soap formed from tall oil acid and a metal of the group of copper, magnesium, calcium, zinc, strontium, barium, tin, lead, chromium, manganese, iron, cobalt and nickel, and a carrying vehicle which acts as a solvent for said soaps.

2. A liquid mixture for producing a resin like protective coating for surfaces consisting essentially of at least two percent of a metal naphthenate soap formed from naphthenic acid and a metal of the group of copper, magnesium, calcium, zinc, strontium, barium, tin, lead, chromium, manganese, iron, cobalt and nickel, a metal tall oil soap formed from tall oil acid and a

metal of the group of copper, magnesium, calcium, zinc, strontium, barium, tin, lead, chromium, manganese, iron, cobalt and nickel, another metal corrosion inhibitor, and a carrying vehicle which acts as a solvent for said soaps and inhibitor.

3. A liquid mixture for producing a resin like protective coating for surfaces consisting essentially of a lead tall oil soap, a zinc naphthenate soap, a calcium naphthenate soap, and a carrying vehicle which acts as a solvent for said soaps.

4. A treating composition for producing a resin-like protective coating comprising 10 to 30% of a metal soap of naphthenic acid in which the metal is selected from the group consisting of copper, magnesium, calcium, zinc, strontium, barium, tin, lead, chromium, manganese, cobalt, and nickel, 10 to 30% of a metal soap of a drying acid selected from the group consisting of tall oil, tung oil, and rosin oil acids, the metal component of which is selected from the group consisting of copper, magnesium, calcium, zinc, strontium, barium, tin, lead, chromium, manganese, cobalt, and nickel, and 40 to 70% of a solvent for the soaps.

5. A treating composition for producing a resin-like protective coating comprising 10 to 30% of a metal soap of naphthenic acid in which the metal is selected from the group consisting of

copper, magnesium, calcium, zinc, strontium, barium, tin, lead, chromium, manganese, cobalt, and nickel, 10 to 30% of a metal soap of a drying acid selected from the group consisting of tall oil, tung oil, and rosin oil acids, the metal component of which is selected from the group consisting of copper, magnesium, calcium, zinc, strontium, barium, tin, lead, chromium, manganese, cobalt, and nickel, 3 to 10% of an inhibitor, and 40 to 70% of a solvent for the soaps.

6. A resin-like protective coating comprising at least 2 percent of a metal soap of naphthenic acid in which the metal is selected from the group consisting of copper, magnesium, calcium, zinc, strontium, barium, tin, lead, chromium, manganese, cobalt, and nickel, and a metal soap of an unsaturated air-drying acid selected from the group consisting of tall oil, tung oil, and rosin oil acids, and mixtures thereof, and in which the metal component is selected from the above metal group.

7. A resin-like protective coating as claimed in claim 6 in which the soaps are present in the ratio of 1 to 3 parts of the naphthenic soap to 1 to 3 parts of the unsaturated drying oil soap.

8. A resin-like protective coating as claimed in claim 7 containing in addition 0.3 to 1 part of another metal corrosion inhibitor.

9. A liquid corrosion inhibiting composition for providing a resin-like protective coating comprising a calcium naphthenate and a zinc naphthenate together totaling at least two percent of the composition a metallic soap formed of tall oil acids, the metallic component of which is selected from the group consisting of copper, magnesium, calcium, zinc, strontium, barium, tin, lead, chromium, manganese, iron, cobalt, nickel, and mixtures thereof, and a carrying vehicle in which said soaps are soluble.

10. A liquid corrosion inhibiting composition for providing a resin-like protective coating comprising a calcium naphthenate and a zinc naphthenate together totaling at least two percent of the composition, a lead tall oil soap, and a carrying vehicle in which said soaps are soluble.

11. A treating composition for producing a resin-like protective coating consisting essentially of a metal soap of naphthenic acid in which the metal is selected from the group consisting of copper, magnesium, calcium, zinc, strontium, barium, tin, lead, chromium, manganese, cobalt, and nickel, a metal soap of an unsaturated drying acid having a relatively high iodine value in which the metal is selected from the group consisting of copper, magnesium, calcium, zinc, strontium, barium, tin, lead, chromium, manganese, cobalt and nickel, each of the soaps being present in amounts greater than 2 percent by weight, a mineral oil and a solvent for said soaps.

HELEN SELLEI BERETVÁS.

#### REFERENCES CITED

The following references are of record in the file of this patent:

#### UNITED STATES PATENTS

| Number       | Name        | Date          |
|--------------|-------------|---------------|
| 1,983,006    | Schladebach | Dec. 4, 1934  |
| 30 2,124,446 | Detwiler    | July 19, 1938 |
| 2,334,071    | Cook        | Nov. 9, 1943  |
| 2,367,462    | Farber      | Jan. 16, 1945 |
| 2,418,075    | Kollen      | Mar. 25, 1947 |
| 2,421,672    | Wilson      | June 3, 1947  |

#### FOREIGN PATENTS

| Number     | Country | Date         |
|------------|---------|--------------|
| 35 681,855 | Germany | Oct. 3, 1939 |